

Jan. 10, 1967

F. W. MEISEL, JR., ET AL  
METHOD FOR EXPLOSION RETICULATION USING  
A NON-INFLAMMABLE LIQUID  
Filed Jan. 27, 1964

3,297,803

Fig. 1



Fig. 2



Fig. 3

INVENTORS.  
FRED W. MEISEL, JR.  
EDGAR ALLAN BLAIR

BY *Sharon T. Hadley*  
ATTORNEY

## 1

3,297,803

METHOD FOR EXPLOSION RETICULATION USING  
A NON-INFLAMMABLE LIQUIDFred W. Meisel, Jr., Media, and Edgar Allan Blair,  
Swarthmore, Pa., assignors to Scott Paper Company,  
Philadelphia, Pa., a corporation of PennsylvaniaFiled Jan. 27, 1964, Ser. No. 340,487  
15 Claims. (Cl. 264—84)

This invention relates to an improved method for treating polymeric foam bodies, more particularly, this invention pertains to reticulation and modification of polymeric foam materials susceptible of undesired changes under explosion reticulation conditions.

Prior art processes for treating foams by explosion techniques have been disclosed in Serial No. 324,578, filed November 18, 1963. Foams represented therein give heretofore unachieved properties although they are in many respect similar to those disclosed in Serial No. 655,368, filed April 26, 1957 and now abandoned. Both of the above-referenced applications are assigned to a common assignee, Scott Paper Company, which is also the assignee of the present application. While the above flame reticulation process represents a significant breakthrough in using an alternative process for foam reticulation, the present process illustrates a further improvement over the flame or explosion process shown in the first-mentioned case.

It has been observed that when certain polymeric, organic foams are subjected to the dewindowing explosion, the foam bodies tend to tear or shatter as well as burn on the surface.

Under proper conditions, the tearing and shattering can be controlled, but it renders the prior art explosive process more cumbersome to use. Decreasing the explosive force by adding more nitrogen generally does not solve the problem under all conditions as the explosion then fails to dewindow the diaphanous faces of foam polyhedrons. Increasing the amount of fuel in the explodable gas mixture, on the other hand, often results in burning. Soft foams or foams which melt easily are especially susceptible to slight variations from the ideal condition. For better understanding of this process the general teaching of the prior art process disclosed in the above Serial No. 324,578 is incorporated herein.

It has now been found that the explosive force results in an improved process over that in Serial No. 324,578 if the process is modified to maintain the brisance needed to dewindow the materials and, at the same time, the brisance is specifically minimized to eliminate the tearing and shattering of the foam. Thus, a novel explosion process is obtained providing exceptionally good controls.

The invention has been accomplished by running the process as in Serial No. 324,578 except that the foam body is soaked in a nonflammable, or nonignitable liquid capable of absorbing the excessive explosive force. Water is the preferred liquid. Others are the fire-resistant hydraulic oils made of monomeric and polymeric phosphorous or silicone derivatives. Mixtures of the above liquids, if compatible, serve equally well. Other nonflammable liquids are obvious to a man skilled in the art. Organic, polymeric foams such as polyurethane, polyvinyl, polyolefin (ethylene), etc. are specific examples within the scope of this invention.

The invention disclosed herein accomplished by a process for reticulating noninflammable liquid-fluid containing open-celled, organic, polymeric foams comprising the steps of: (a) introducing into a gas-confining, foam-containing zone a mixture of oxygen-containing gas and a gas explosively combustible in contact with oxygen; (b) permeating the previously wetted foam material with said

## 2

gas composition for a time sufficient to insure a distribution of sufficient quantity of the gas mixture in the foam material; (c) igniting the gas mixture to obtain a flame propagation throughout the wetted foam material; and (d) recovering a reticulated foam material. In general, the above foam will contain from about 6 to about 125 p.p.i.; in the preferred embodiment, of from about 10 to about 100 p.p.i.; or, in the more preferred embodiment, 10 to 45 p.p.i.

- 10 In another aspect, this invention is accomplished by a process for dewindowing a polyurethane foam material having partially-communicating cells comprising the steps of: (a) introducing into a gas-confining, foam containing zone a foam material wetted with a nonignitable liquid, (b) thereafter introducing in said zone a mixture of oxygen-containing gas and a gas explosively combustible in contact with oxygen; (c) permeating the foam material with said gas composition for a time sufficient to insure a distribution of sufficient quantity of the gas mixture in the foam material; (d) igniting the gas mixture to obtain a flame propagation throughout the wetted foam material; and (e) recovering a reticulated foam material.
- 15 In a further aspect, this invention has been accomplished by a process for preparing reticulated, organic, polymeric foam body having a three-dimensional strand network joined at the nexuses wherein the strands define the polygonal faces of a foam building-block polyhedron, said polyhedron having a majority, but less than all of the faces defined by said strand network, and a unitary membrane joined to the defining strands, said individual polyhedrons joined together by common nexuses and strands making up the foam body, wherein the membraneless faces are in open communication with other cells' open faces, said body containing a dispersed liquid fluid
- 20 substantially nonignitable under explosive flame conditions, the process comprising the steps of (a) introducing into a gas-confining zone the fluid-containing body; (b) permeating the gas and foam-body confining zone by introducing into said zone a mixture of oxygen-containing gas and a gas explosively combustible in contact with oxygen, the amount of oxygen in the mixture being in excess of at least that amount of oxygen introduced in the mixture in the form of air; (c) kneading said foam material to insure a further distribution of said fluid and explosive
- 25 gas mixture; (d) igniting the gas mixture to obtain a flame propagation in the foam material (e) recovering a reticulated foam material and (f) repeatedly subjecting the foam material to said modified explosive treatment.

25 In still another aspect, this invention has been accomplished by a process for producing a membrane-free foam body comprising the steps of (a) introducing into a gas-confining zone a foam body containing a liquid fluid noninflammable under explosive flame conditions; (b) evacuating the gas-confining, foam-body containing zone; (c) introducing into the gas-confining zone a liquid fuel without bringing said liquid fuel in contact with said liquid fluid-containing foam body, said liquid fuel being characterized by a high vapor pressure at standard conditions; (d) maintaining the temperature in the confined zone at a suitable level at which the vapor pressure of the liquid fuel is sufficient to permit the fuel to exist in gas phase to form an explodable mixture in the presence of oxygen; (e) introducing a mixture of oxygen-containing gas into said gas-confining zone; (f) permeating said foam body with the oxygen-containing gas and vapor from the evaporating liquid; (g) igniting said combustible mixture; and (h) recovering the foam material.

30 In the drawing, FIGURE 1 diagrammatically represents an illustrative process and several variations of the process employing the present invention. FIGURE 2 is a greatly enlarged perspective view of an individual

polymeric foam cell illustrating the skeletal structure and remaining cell membranes. FIGURE 3 is a greatly enlarged perspective view of an individual reticulated polymeric foam cell illustrating the skeletal structure shown in FIGURE 2 which remains after the removal of the cell membranes in accordance with the process of the invention.

The novel aspect of controlling the reticulation is accomplished by the above process wherein said liquid, being selected from at least one member of the group consisting of lower alkyl ethers of from 1 to 4 carbon atoms, at least one of the alkyls having 2 carbon atoms when the other alkyl is  $-\text{CH}_3$ , lower alkyl alcohols of from 1 to 4 carbon atoms, said compounds being further characterized by high vapor pressures at normal conditions. A successful reticulation is characterized by the fact that the diaphanous membranes of said foam material are absent from the final product in the areas of the explosive effect.

5 10

The bag may also be connected to a vacuum source to evacuate air from the foam. Repeating the evacuating operation a few times insures the ready distribution of the explosive gas.

5 15

The following examples are included to illustrate the various facets of the invention. These examples are to be construed with reference to the above discussion and claims, and are not intended to limit the broader scope of the invention.

#### EXAMPLE 1

A block of flexible polymeric polyether polyurethane having a density of 1.0 p.c.f. and 45 p.p.i. (pores per inch), made by reacting a mixture of polyether triol and diol with toluene diisocyanate and water in a conventional one-shot process, but obtaining a part of the blowing with "Freon 11," is treated according to the procedure outlined above (also described in Serial No. 324,578) with several fuel gases.

Results:

| Run          | Fuel           | Gas comp., <sup>1</sup> vol. percent |      | Foam wt. loss, percent | Tens., p.s.i. | Elong., percent | Tear, lbs./in. | Comp. Set | Comp./Defl. |     |     | Reticulation |
|--------------|----------------|--------------------------------------|------|------------------------|---------------|-----------------|----------------|-----------|-------------|-----|-----|--------------|
|              |                | O <sub>2</sub>                       | Fuel |                        |               |                 |                |           | 25%         | 50% | 66% |              |
| 1.....       | Propane.....   | 63                                   | 7    | 4.8                    | 19.1          | 400             | 2.7            | 26        | .12         | .12 | .16 | Complete.    |
| 2.....       | Acetylene..... | 37                                   | 15   | 2.0                    | 13.9          | 315             | 2.0            | 20        | .17         | .20 | .27 | Do.          |
| 3.....       | do.....        | 70                                   | 15   | 6.0                    | 16.0          | 380             | 2.4            | 24        | .12         | .14 | .17 | Do.          |
| Control..... |                |                                      |      |                        | 9.9           | 165             | 1.3            | 11        | .29         | .30 | .37 | None.        |

<sup>1</sup> Balance N<sub>2</sub>.

In order to aid the interconnection of the cells, the membranes may also be mechanically ruptured without removing them, such as by wringing or swelling the foam in a solvent and then breaking the weakened foam. Still other methods may be used to rupture the membranes (without being removed from the foam body), but this step is generally for the purpose of enabling ready permeating of the water or the noninflammable fluid and the explosive gas mixture.

Various gases are useful as the explosive (combustion) force. Acetylene and propane are the preferred gases. Other gases suitable for the present process are selected from at least one member of the group methane, ethane, butane, ethylene—in general exemplifying the hydrocar-

Foam properties are determined in all examples by ASTM Methods D1564-54T.

#### EXAMPLE 2

45 35 40 45

A block of polymeric polyether polyurethane foam, generally similar to the material of Example 1 is used, except that a different polyether is employed. This polyether is obtained from Witco Chemical Co., Chicago, Ill. and is sold under the trade-mark "Formez" G-26-9 and is characterized by an hydroxyl number of about 110 with an acid number of about 0.06 and an unsaturated milli-equivalent per gram of 0.006, and is treated according to the procedure of Example 1. Density of the foam is 1.02; pore size is 45 p.p.i.

| Run          | Fuel           | Gas comp., <sup>1</sup> vol. percent |      | Foam wt. loss, percent | Tens., p.s.i. | Elong., percent | Tear, lbs./in. | Comp. Set | Comp./Defl. |     |     | Reticulation |
|--------------|----------------|--------------------------------------|------|------------------------|---------------|-----------------|----------------|-----------|-------------|-----|-----|--------------|
|              |                | O <sub>2</sub>                       | Fuel |                        |               |                 |                |           | 25%         | 50% | 66% |              |
| 1.....       | Propane.....   | 63                                   | 7    | (2)                    | (2)           | (2)             | (2)            | (2)       | (2)         | (2) | (2) | Complete.    |
| 2.....       | Acetylene..... | 37                                   | 15   | 3.2                    | 18.0          | 240             | 1.8            | 10        | .10         | .12 | .22 | Do.          |
| 3.....       | do.....        | 70                                   | 15   | (3)                    | 22.7          | 305             | 2.1            | 19        | .06         | .07 | .12 | Do.          |
| Control..... |                |                                      |      |                        | 6.5           | 155             | 1.3            | 13        | .11         | .14 | .21 | None.        |

<sup>1</sup> Balance N<sub>2</sub>.

<sup>2</sup> Sample torn apart.

<sup>3</sup> Sample torn.

bon group—as well as the above-mentioned acetylene and propane. Other materials useful in the reaction are hydrogen, hydrogen sulfide, ethylene oxide, methylether, and liquids, such as methylethylether, the low-boiling-point alkyl ethers, and alcohols such as methyl, ethyl and isopropyl alcohol.

Gases used in the explosion are controlled as to their ratios and rate by gauges and flowmeters located at supply sources. Generally, the supply sources are sufficiently far removed from the explosion zone.

The explosive zone to which the gases are fed via the supply line, consists of a polyethylene bag containing a foam block and an ignition source to initiate the explosion.

65

This is very soft foam and considerable difficulty with tearing is encountered; otherwise, results are generally similar to those obtained with the foam of Example 1.

#### EXAMPLE 3

70 75

A block of flexible polyurethane adipate polyester foam of a density of 1.9 pounds per cubic foot and of 45 p.p.i. is wetted with water. A portion of the wet block is exposed to conditions created by exploding a gaseous mixture of acetylene and oxygen of 1 part acetylene to 2 and 2.5 parts of oxygen and fed to the system at a rate of 35 cubic feet per minute for 3 minutes. The foam is effectively reticulated without the surface scorching obtained

when the foam is subjected to the explosive force in the dry state under the same conditions.

#### EXAMPLE 4

Blocks of unreticulate foams which are of the same block as in Example 2 are subjected to the same explosion treatment except that the foam is immersed in water, squeezed to remove excess water and then reticulated. The foam bodies, when treated with explosive flame display substantially no tearing.

#### EXAMPLE 5

A large block of polyurethane foam is prepared by a conventional one-shot foaming process using an 80-20 isomeric mixture of 2,4- and 2,6-toluene diisocyanate and castor oil.

Specimens of 6" x 6" x 3" are cut from the large block and exposed to conditions created by igniting an explosive mixture of acetylene and oxygen. An effectively reticulated foam is obtained; however, it is somewhat soft and gummy. Wetting another specimen of the same foam with water and then subjecting it to an exploding acetylene-oxygen mixture considerably diminishes the gumminess of the foam.

#### EXAMPLE 6

A number of specimens from a 45 p.p.i. polyurethane adipate polyester foam are subjected to an explosive force generated by hydrogen sulfide oxygen-nitrogen mixture. The data below illustrate the results.

Above experiments are then carried out by wetting the foam sample with water. Rupturing or tearing is avoided and burning eliminated if the foam block is wetted enough to absorb the excess energy. This example demonstrates that a highly brisant explosion such as obtained by a 50-50 mixture of the above gas components may effectively be modified by using water as energy-dissipating media.

Foams treated under the conditions employed above include the previously mentioned ethers, esters and castor oil foams. By means of this modified procedure rigid polyether foams have also been successfully reticulated.

In practicing the invention foams of various pore size are used. Applying the explosion treatment of foams having different pore sizes generally requires some adjustment in the fuel-gas, oxygen-containing gas and water variables. From a practical point of view the first two variables are first explored to see if the desired control can be easily achieved; then, if the first two variables do not readily give the desired result the moistening step is used to achieve better control. However, it is to be understood that using the noninflammable fluid at any desired condition affords more precise process control and facilitates the determination of the optimum conditions.

25 What is claimed is:

1. A process for removing diaphanous membranes from organic, polymeric foams capable of being permeated with an explodable mixture of fuel gas and oxygen comprising the steps of:

30 (a) applying a dispersed noninflammable fluid to the

#### HYDROGEN SULFIDE

| Run    | Gas mixture, vol. percent |                |                | Total gas flow rate, c.f.h. | Orig. wt., grams | Wt. after treatment, grams | Retic.                     |
|--------|---------------------------|----------------|----------------|-----------------------------|------------------|----------------------------|----------------------------|
|        | H <sub>2</sub> S          | O <sub>2</sub> | N <sub>2</sub> |                             |                  |                            |                            |
| 1----- | 40                        | 60             | 0              | 7.5                         | 53.6             | 52.8                       | Compl.                     |
| 2----- | 30                        | 70             | 0              | 10.0                        | 52.3             | 51.0                       | Compl.                     |
| 3----- | 23.1                      | 76.9           | 0              | 13.0                        | 51.1             | 50.3                       | Compl.                     |
| 4----- | 60                        | 40             | 0              | 10.0                        | 52.5             | 52.2                       | Incompl.                   |
| 5----- | 70                        | 30             | 0              | 10.0                        | 50.6             | -----                      | Complete; specimen burned. |

The above experiments are then carried out by slightly wetting the specimens. If excess water (after dipping and slight squeezing) is present the explosion is considerably less effective. This indicates that water is a good fluid for modifying the explosive force used in foam reticulation.

#### EXAMPLE 7

A number of specimens from a 45 p.p.i. polyurethane adipate polyester foam are subjected to an explosive force generated by ethylene oxide-oxygen mixture according to the procedure described above. The data below illustrate the results.

internal and external surfaces of said foam body;  
 (b) introducing said explodable fuel-oxygen mixture into said foam body;  
 (c) creating an explosive flame propagation in the foam material; and  
 (d) recovering the product.

2. A process for reticulating open-celled, organic, polymeric foams comprising the steps of:

(a) applying a dispersed noninflammable liquid fluid to the internal and external surfaces of a body of open-celled, organic, polymeric foam material;  
 (b) introducing a mixture of oxygen-containing gas and

#### ETHYLENE OXIDE

| Run    | Gas Mixture, vol. percent |                |                | Total gas flow rate, c.f.h. | Orig. wt., grams | Comments                                                       |
|--------|---------------------------|----------------|----------------|-----------------------------|------------------|----------------------------------------------------------------|
|        | E.O.                      | O <sub>2</sub> | N <sub>2</sub> |                             |                  |                                                                |
| 1----- | 100                       | 0              | 0              | 5                           | 50.3             | No explosion.                                                  |
| 2----- | 28.5                      | 71.5           | 0              | 17.5                        | 50.5             | Bad rupture; complete reticulation.                            |
| 3----- | 20.0                      | 80             | 0              | 2.5                         | 49.7             | Very slight explosion; burning.                                |
| 4----- | 10.0                      | 90.0           | 0              | 50                          | 52.4             | No explosion.                                                  |
| 5----- | 50.0                      | 50.0           | 0              | 10                          | 52.3             | Bad rupture; complete reticulation.                            |
| 6----- | 75.0                      | 25.0           | 0              | 10.5                        | 53.0             | Burning; incomplete reticulation.                              |
| 7----- | 28.5                      | 71.5           | 0              | 17.5                        | 51.2             | Explosion very loud; complete reticulation.                    |
| 8----- | 30.0                      | 50.0           | 0              | 10                          | 51.3             | Very loud explosion (brisant); complete reticulation; tearing. |

- a gas explosively combustible in contact with oxygen into a gas-confining zone;
- (c) permeating the previously wetted foam material with said gas composition for a time sufficient to insure a distribution of the gas mixture in the foam material;
- (d) igniting the gas mixture to obtain a flame propagation in the foam material; and
- (e) recovering a reticulated foam material.

3. A process for flame dewindowing of organic, polymeric foam material having partially communicating cells comprising the steps of:

- (a) applying a dispersed noninflammable liquid fluid to the internal and external surfaces of a body of said foam;
- (b) introducing said body of foam material and a mixture of oxygen-containing gas, into a gas-confining zone, and thereafter introducing into the same zone a gas explosively combustible in contact with oxygen, the amount of oxygen present being in excess of at least about that amount of oxygen introduced in the mixture in form of air;
- (c) permeating the foam material with said gas composition for a time sufficient to insure a distribution of the explosive gas in the foam material;
- (d) igniting the gas mixture to obtain an explosive reaction of the oxygen and combustible gas in the gas-confining zone; and
- (e) recovering a reticulated foam material.

4. A process for dewindowing polyurethane foam material having partially communicating cells comprising the steps of:

- (a) applying a dispersed noninflammable liquid fluid to the internal and external surfaces of a body of polyurethane foam material;
- (b) introducing the wetted foam material and a mixture of oxygen-containing gas and a gas explosively combustible in contact with oxygen into a gas-confining zone;
- (c) permeating the foam material with said gas composition for a time sufficient to insure a distribution of the gas mixture in the foam material;
- (d) igniting the gas mixture to obtain a flame propagation in the foam material and;
- (e) recovering a reticulated foam material.

5. The process according to claim 4 wherein the foam material is polyurethane polyester foam.

6. The process according to claim 4 wherein the foam material is polyurethane polyether foam.

7. The process according to claim 2 wherein the wetted foam material is a polyvinylchloride.

8. A process for preparing reticulated, organic, polymeric foam from a foam body having a three-dimensional strand network joined at the nexuses wherein the strands define the polygonal faces of an individual foam building block polyhedron, said polyhedron having a majority but less than all of the faces defined by said strand network and a unitary membrane joined to the defining strands, said individual polyhedrons joined together by common nexuses and strands making up the foam body, wherein the membraneless faces are in open communication with other cells' open faces, the process comprising the steps of:

- (a) applying a dispersed noninflammable liquid fluid to the internal and external surfaces of said foam body;
- (b) introducing into a gas-confining zone said fluid-containing body;
- (c) permeating the gas- and foam body-confining zone by introducing into said zone a mixture of oxygen-containing gas and a gas explosively combustible in contact with oxygen;
- (d) kneading said foam material to insure a further distribution of said fluid and explosive gas mixture;

75

- (e) igniting the gas mixture to obtain a flame propagation throughout the foam material; and
- (f) recovering a reticulated foam material; and
- (g) repeatedly subjecting the foam material to said explosive treatment.

9. A process for producing a membrane-free organic, polymeric foam body comprising the steps of:

- (a) applying a dispersed noninflammable liquid fluid to the internal and external surfaces of a body of open-celled, organic, polymeric foam materials;
- (b) introducing into a gas-confining zone a foam body containing a liquid fluid non-inflammable under explosive flame conditions;
- (c) evacuating gas-confining foam body-containing zone;
- (d) introducing into the gas-confining zone a liquid without bringing said liquid in contact with said foam body, said liquid fuel being characterized by a high vapor pressure standard conditions;
- (e) maintaining the temperature in the confined zone at a suitable level at which the vapor pressure of the liquid fuel is sufficient to permit the fuel to exist in gas phase at a concentration to form an explosive mixture in the presence of oxygen;
- (f) introducing a mixture of oxygen-containing gas into said gas-confining zone;
- (g) permeating said foam body with the oxygen-containing gas and vapor from the evaporating liquid;
- (h) igniting said combustible mixture; and
- (i) recovering the foam material.

10. An improved process for producing reticulated, organic, polymeric foam materials comprising the steps of:

- (a) taking an open-celled foam of from 6 to 125 pores per linear inch and wetting it throughout with water;
- (b) evacuating a gas-confining and wet foam material-containing zone;
- (c) introducing into the evacuated gas-confining zone a mixture of oxygen-enriched gas and a gas explosively combustible in contact with oxygen, said combustible gas being selected from at least one member of the group consisting of hydrogen, hydrogen sulfide, acetylene, ethylene, methane, ethane, propane, utane ethylene oxide and methylether;
- (d) permeating said foam material with said explosive gas mixture;
- (e) igniting said gas mixture; and
- (f) recovering a reticulated product.

11. The process according to claim 10 wherein the gas is acetylene and the foam material is polyether polyurethane.

12. The process according to claim 10 wherein the gas is ethylene oxide.

13. A process for producing reticulated foam materials comprising the steps of:

- (a) taking an open-celled foam of from 6 to 125 pores per linear inch and wetting it throughout with water;
- (b) evacuating a gas-confining and wet foam material-containing zone;
- (c) introducing into the gas-confining zone a liquid without bringing said liquid in contact with said foam body, said liquid being selected from at least one member from the group consisting of lower alkyl-ethers of from 1 to 4 carbon atoms, at least one of the alkyls having 2 carbon atoms when the other is  $-\text{CH}_3$ ; and lower alkyl alcohols, said compounds being further characterized by high vapor pressures at normal conditions;
- (d) maintaining the temperature in the confined zone at a suitable level at which the vapor pressure of the liquid fuel is sufficient to permit the fuel to exist in gas phase in a concentration to form an explosive mixture in the presence of oxygen; but at a temperature lower than the boiling point of water;
- (e) introducing a mixture of oxygen-containing gas into said liquid and gas-confining zone;

- (f) permeating said foam body with the oxygen-containing gas and vapor from the evaporating liquid;
  - (g) igniting said combustible mixture, said oxygen-vapor mixture being characterized by a flame front capable of reticulating the diaphanous membranes of said foam material; and
  - (h) recovering the foam material.
14. The process according to claim 13 wherein the liquid is methylethylether.

15. The process according to claim 14 wherein the liquid is isopropylalcohol.

**References Cited by the Examiner**

UNITED STATES PATENTS

2,961,710 11/1960 Stark ----- 264—54  
3,175,025 3/1965 Geen et al. ----- 264—321 XR

ALEXANDER H. BRODMERKEL, *Primary Examiner.*

P. E. ANDERSON, *Assistant Examiner.*